



US007129283B2

(12) **United States Patent**  
**Wang et al.**

(10) **Patent No.:** **US 7,129,283 B2**  
(45) **Date of Patent:** **Oct. 31, 2006**

(54) **BINDERS CONTAINING AN EPOXY RESIN, AN ESTER OF A FATTY ACID, AND A FLUORINATED ACID**

(75) Inventors: **Xianping Wang**, Dublin, OH (US); **H. Randall Shriver**, Columbus, OH (US); **Jorg Kroker**, Powell, OH (US)

(73) Assignee: **Ashland Licensing and Intellectual Property LLC**, Dublin, OH (US)

(\*) Notice: Subject to any disclaimer, the term of this patent is extended or adjusted under 35 U.S.C. 154(b) by 335 days.

(21) Appl. No.: **10/627,471**

(22) Filed: **Jul. 25, 2003**

(65) **Prior Publication Data**

US 2005/0020725 A1 Jan. 27, 2005

(51) **Int. Cl.**

**C08G 67/02** (2006.01)

**C08K 5/098** (2006.01)

**B22C 1/22** (2006.01)

(52) **U.S. Cl.** ..... **523/139**; 523/141; 523/144; 523/145; 528/405; 264/83; 164/16; 524/284; 524/612

(58) **Field of Classification Search** ..... 523/139, 523/141, 144, 145; 528/405; 264/83; 164/16; 524/284, 612

See application file for complete search history.

(56)

**References Cited**

**U.S. PATENT DOCUMENTS**

|              |   |         |                        |         |
|--------------|---|---------|------------------------|---------|
| 3,107,403 A  | * | 10/1963 | Moore .....            | 164/16  |
| 3,145,438 A  | * | 8/1964  | Kottke et al. .....    | 164/16  |
| 4,518,723 A  |   | 5/1985  | Woodson .....          | 523/466 |
| 4,526,219 A  |   | 7/1985  | Dunnivant et al. ..... | 164/16  |
| 4,806,576 A  |   | 2/1989  | Woodson .....          | 523/139 |
| 6,136,888 A  |   | 10/2000 | Torbus et al. .....    | 523/142 |
| 6,465,542 B1 |   | 10/2002 | Torbus et al. .....    | 523/143 |
| 6,664,310 B1 | * | 12/2003 | Chen et al. .....      | 523/139 |

**FOREIGN PATENT DOCUMENTS**

DE 19727540 A1 3/1998

\* cited by examiner

*Primary Examiner*—Kriellion Sanders

(74) *Attorney, Agent, or Firm*—David L. Hedden

(57) **ABSTRACT**

This invention relates to foundry binder systems, which cure in the presence of sulfur dioxide and an oxidizing agent, comprising (a) an epoxy resin; (b) an ester of a fatty acid; (c) a fluorinated acid, preferably hydrofluoric acid; (d) an effective amount of an oxidizing agent; and (e) no ethylenically unsaturated monomer or polymer. The foundry binder systems are used for making foundry mixes. The foundry mixes are used to make foundry shapes (such as cores and molds) which are used to make metal castings, particularly ferrous castings.

**12 Claims, No Drawings**

## 1

**BINDERS CONTAINING AN EPOXY RESIN,  
AN ESTER OF A FATTY ACID, AND A  
FLUORINATED ACID**

FIELD OF THE INVENTION

This invention relates to foundry binder systems, which cure in the presence of sulfur dioxide and an oxidizing agent, comprising (a) an epoxy resin; (b) an ester of a fatty acid; (c) a fluorinated acid, preferably hydrofluoric acid; (d) an effective amount of an oxidizing agent; and (e) no ethylenically unsaturated monomer or polymer. The foundry binder systems are used for making foundry mixes. The foundry mixes are used to make foundry shapes (such as cores and molds) which are used to make metal castings, particularly ferrous castings.

DESCRIPTION OF THE RELATED ART

In the foundry industry, one of the procedures used for making metal parts is "sand casting". In sand casting, disposable molds and cores are fabricated with a mixture of sand and an organic or inorganic binder. The foundry shapes are arranged in core/mold assembly, which results in a cavity into which molten metal will be poured. After the molten metal is poured into the assembly of molds and cores and cools, the metal part formed by the process is removed from the assembly. The binder is needed so the molds and cores will not disintegrate when they come into contact with the molten metal.

Two of the prominent fabrication processes used in sand casting are the no-bake and the cold-box processes. In the no-bake process, a liquid curing catalyst or co-reactant is mixed with an aggregate and binder to form a foundry mix before shaping the mixture in a pattern. The foundry mix is shaped by putting it into a pattern and allowing it to cure until it is self-supporting and can be handled. In the cold-box process, a gaseous curing catalyst or co-reactant is passed through a shaped mixture (usually in a corebox) of the aggregate and binder to cure the mixture.

A cold-box process widely used in the foundry industry for making cores and molds is the "SO<sub>2</sub> cured epoxy/acrylate system". In this process, a mixture of a hydroperoxide (usually cumene hydroperoxide), an epoxy resin, a multifunctional acrylate, typically a coupling agent, and optional diluents, are mixed into an aggregate (sand) and compacted into a specific shape, typically a core or mold. Sulfur dioxide (SO<sub>2</sub>), optionally diluted with nitrogen or another inert gas, is blown into the binder/aggregate shape. The shape is instantaneously hardened and can be used immediately in a foundry core/mold system. In this binder system, the acrylate component must be kept separate from the hydroperoxide until the binder is applied to sand, otherwise, free radical polymerization of the acrylate component will begin prematurely and render the binder useless.

German Patent Application DE 197 27 540 discloses examples of epoxy-acrylic foundry binders containing methyl-, ethyl- and propyl-esters of oleic acid, which are cured with sulfur dioxide in the presence of a free radical initiator.

BRIEF SUMMARY OF THE INVENTION

The subject invention relates to foundry binder systems, which cure in the presence of gaseous sulfur dioxide and an oxidizing agent, comprising:

## 2

- (a) 45 to 80 parts by weight of an epoxy resin;  
(b) 5 to 40 parts of an ester of a fatty acid;  
(c) 0.05 to 3 parts of a fluorinated acid;  
(d) an effective amount of an oxidizing agent; and  
(e) 0 parts of an ethylenically unsaturated monomer or polymer.

wherein (a), (b), (c), and (d) are separate components or mixed with another of said components, and where said parts by weight are based upon 100 parts of binder.

10 It has been found that addition of the fluorinated acid to an acrylate-free binder provides foundry shapes that have better tensile strength development and humidity resistance than foundry shapes made with binders that do not contain the fluorinated acid. Tests have also shown that the foundry shapes, made with these binders, have better tensile strength development and humidity resistance than those made with similar binders containing an acrylate and no fluorinated acid. This is beneficial in the casting of both light metal (e.g. aluminum) and ferrous parts.

15 20 Another advantage of the binder, because it is acrylate-free, is that all of the components of the binder can be sold and used in one package. This simplifies the customer's binder storage and handling operations.

The foundry binders are used for making foundry mixes. 25 The foundry mixes are used to make foundry shapes, such as cores and molds, which are used to make metal castings.

DETAILED DESCRIPTION OF THE  
INVENTION

30 The detailed description and examples will illustrate specific embodiments of the invention will enable one skilled in the art to practice the invention, including the best mode. It is contemplated that many equivalent embodiments 35 of the invention will be operable besides these specifically disclosed. All percentages are percentages by weight unless otherwise specified.

An epoxy resin is a resin having an epoxide group, i.e.,



40 45 such that the epoxide functionality of the epoxy resin (epoxide groups per molecule) is equal to or greater than 1.9, typically from 2.0 to 4.0.

50 Examples of epoxy resins include (1) diglycidyl ethers of bisphenol A, B, F, G and H, (2) halogen-substituted aliphatic epoxides and diglycidyl ethers of other bisphenol compounds such as bisphenol A, B, F, G, and H, and (3) epoxy novolacs, which are glycidyl ethers of phenolic-aldehyde novolacs, (4) cycloaliphatic epoxy resins, and (5) mixtures thereof.

55 60 Epoxy resins (1) are made by reacting epichlorohydrin with the bisphenol compound in the presence of an alkaline catalyst. By controlling the operating conditions and varying the ratio of epichlorohydrin to bisphenol compound, products of different molecular weight can be made. Epoxy resins of the type described above based on various bisphenols are available from a wide variety of commercial sources.

65 Examples of epoxy resins (2) include halogen-substituted aliphatic epoxides, diglycidyl ethers of other bisphenol

compounds such as bisphenol A, B, F, G, and H, and epoxy novolac resins. Examples of halogen-substituted aliphatic epoxides include epichlorohydrin, 4-chloro-1,2-epoxybutane, 5-bromo-1,2-epoxypentane, 6-chloro-1,3-epoxyhexane and the like.

Examples of epoxy novolacs (3) include epoxy cresol and epoxy phenol novolacs, which are produced by reacting a novolac resin (usually formed by the reaction of orthocresol or phenol and formaldehyde) with epichlorohydrin, 4-chloro-1,2-0.4 epoxybutane, 5-bromo-1,2-epoxypentane, 6-chloro-1,3-epoxyhexane and the like.

Examples of cycloaliphatic epoxy resins include any aliphatic, cycloaliphatic, or mixed aliphatic-cycloaliphatic epoxide having any aliphatic groups, and further includes aliphatic epoxy resins having aromatic groups, i.e. mixed aliphatic-aromatic epoxy resins. The aliphatic epoxy resin may contain monomeric epoxide compounds in admixture with polymeric epoxide compounds. The most preferred aliphatic epoxy resins are represented by the following structural formulae:



(I)

where "n"  $\geq 1$  and "m" is a whole number, typically from 1 to 4, preferably from 2-3, or



(II)

where "n"  $\geq 1$ .

R in structures I and II is predominantly aliphatic in nature, but may contain oxygen functionality as well as mixed aliphatic-aromatic groups. Typically, R is selected from the group consisting of alkyl groups, cycloalkyl groups, mixed alkyl-cycloaliphatic groups, and substituted alkyl groups, cycloalkyl groups, or alkyl-cycloaliphatic groups, where the substituents include, for example, ether, carbonyl, and carboxyl groups.

Specific examples of aliphatic epoxy resins include 3,4-epoxycyclohexylmethyl-3,4-epoxycyclohexane carboxylate; vinylcyclohexene dioxide; 2-(3,4-epoxycyclohexyl-5,5-spiro-3,4-epoxy) cyclohexane-meta-dioxane; bis-(3,4-epoxycyclohexyl) adipate; 1,2-epoxy-p-vinylcyclohexene; limonene dioxide; limonene monoxide; and hydrogenated bisphenol diglycidyl ethers.

Preferably used are epoxy resins having an average epoxide functionality of at least 2.1 to 3.5, preferably from about 2.3 to about 3.0. Particularly preferred are epoxy resins having an average weight per epoxy group of 165 to 200 grams/equivalents.

Although it is contemplated that any esters of a fatty acid can be used in this invention, preferably used are esters of fatty acids where the fatty acid used to prepare the ester has a carbon chain of 12 carbon atoms or more, particularly 12-22 carbon atoms. Preferably the ester group of the ester of the fatty acid has 1 to 8 carbon atoms. The esters of the fatty acids can be readily prepared by transesterification of

fats and oils of plant or animal origin, which are normally available in the form of triglycerides or can be prepared by esterification of fatty acids obtained from such fats and oils.

Rapeseed oil methyl ester is a typical example of an ester derived from plant oil; it is a suitable solvent, particularly since it is available at low cost in the form of diesel fuel. But the esters of other plant oils, such as soybean oil, linseed oil, sunflower oil, peanut oil, tung oil, palm kernel oil, coconut oil, castor oil and/or olive oil, can also be used. In addition, marine animal oil, tallow oil, and animal fats can also serve as starting materials for alkyl esters that are to be used according to this invention.

The oxidizing agent is a peroxide and/or hydroperoxide. Examples include ketone peroxides, peroxy ester free radical initiators, alkyl oxides, chlorates, perchlorates, and perbenzoates. Preferably, however, the free radical initiator is a hydroperoxide or a mixture of peroxide and hydroperoxide. Hydroperoxides particularly preferred in the invention include t-butyl hydroperoxide, cumene hydroperoxide, paramenthane hydroperoxide, etc. The organic peroxides may be aromatic, aliphatic, or mixed aromatic-aliphatic peroxides.

Examples of useful diacyl peroxides include benzoyl peroxide, lauroyl peroxide and decanoyl peroxide. Examples of mixed aromatic-aliphatic and aliphatic peroxides respectively include dicumyl peroxide and di-t-butyl peroxide.

Solvents may also be added to the binder formulation. Typically, a solvent is used to reduce the viscosity of the binder, such that the resulting viscosity of the epoxy resin component is less than 1,000 centipoise, preferably less than 400 centipoise. Generally, the total amount of solvent is used in an amount of 0 to 25 weight percent based upon the total weight of the epoxy resin. Solvents that can be used include polar solvents, such as liquid dialkyl esters, e.g. dialkyl phthalate of the type disclosed in U.S. Pat. No. 3,905,934, and other dialkyl esters such as dimethyl glutarate, dimethyl succinate, dimethyl adipate, and mixtures thereof. Suitable aromatic solvents are benzene, toluene, xylene, ethylbenzene, and mixtures thereof. Preferred aromatic solvents are mixed solvents that have an aromatic content of at least 90% and a boiling point range of 138° C. to 232° C. Suitable aliphatic solvents include kerosene.

The binder may also contain a silane coupling agent having the following general formula:



wherein R' is a hydrocarbon radical and preferably an alkyl radical of 1 to 6 carbon atoms and R is an alkyl radical, an alkoxy-substituted alkyl radical, or an alkyl-amine-substituted alkyl radical in which the alkyl groups have from 1 to 6 carbon atoms. The silane is preferably added to the binder in amounts of 0.01 to 2 weight percent, preferably 0.1 to 0.5 weight percent based on the weight of the binder.

Polyols such as phenolic resins, polyester resins, amine polyols, polyester polyols, and polyether polyols can also be used in the foundry binder.

Phenolic resins include phenolic resole resins, particularly benzylidene phenolic resole resins, including alkoxy-modified benzylidene phenolic resole resins. Benzylidene phenolic resins, or alkoxyated versions thereof,

are well known in the art, and are specifically described in U.S. Pat. Nos. 3,485,797 and 4,546,124.

Polyether polyols are prepared by reacting an alkylene oxide with a polyhydric alcohol in the presence of an appropriate catalyst such as sodium methoxide according to methods well known in the art.

The polyester polyols may be aliphatic and/or aromatic polyester polyols. These polyols generally having a hydroxyl number from about 200 to 2,000, preferably from 700 to 1200, and most preferably from 250 to 600 mg KOH/g.

The binder contains a fluorinated acid. Examples of fluorinated acids include hydrofluoric acid, ammonium fluoride, tris-hydrofluoric acid, ammonium bifluoride, potassium bifluoride, tetrafluoroboric acid, hexafluorophosphoric acid, hexafluorosilicic acid, N,N-diisopropyl-amine-tris (hydrogenfluoride), and N,N'-dimethyl-2-imidazolidone-hexakis(hydrogenfluoride). Preferably, the fluorinated acid is hydrofluoric acid, most preferably an aqueous solution of hydrofluoric acid, containing from 10 to 90 weight percent water, preferably 30 to 60 weight percent water.

The components of the binder can be combined as one component and added to the foundry aggregate, or can be added separately or in various combinations.

It will be apparent to those skilled in the art that other additives such as silanes, silicones, release agents, defoamers, wetting agents, etc. can be added to the aggregate, or foundry mix. The particular additives chosen will depend upon the specific purposes of the formulator.

Typically, the amounts of the components used in the binder system are from 45 to 80 parts by weight of epoxy resin, preferably from 50 to 70 parts by weight; from 5 to 40 parts by weight of an ester of a fatty acid, preferably from 15 to 30 parts by weight; from 0.05 to 3 parts by weight of a fluorinated acid, preferably from 0.05 to 1.0 parts by weight; and from 10 to 40 parts by weight of oxidizing agent, preferably from parts by weight, wherein the weight percents are based upon 100 parts of the binder system.

Various types of aggregate and amounts of binder are used to prepare foundry mixes by methods well known in the art. Ordinary shapes, shapes for precision casting, and refractory shapes can be prepared by using the binder systems and proper aggregate. The amount of binder and the type of aggregate used are known to those skilled in the art. The preferred aggregate employed for preparing foundry mixes is sand wherein at least about 70 weight percent, and preferably at least about 85 weight percent, of the sand is silica. Other suitable aggregate materials for ordinary foundry shapes include zircon, olivine, aluminosilicate, chromite sands, and the like.

In ordinary sand type foundry applications, the amount of binder is generally no greater than about 10% by weight and frequently within the range of about 0.5% to about 7% by weight based upon the weight of the aggregate. Most often, the binder content for ordinary sand foundry shapes ranges from about 0.6% to about 5% by weight based upon the weight of the aggregate in ordinary sand-type foundry shapes.

The foundry mix is molded into the desired shape by ramming, blowing, or other known foundry core and mold making methods. The shape is then cured almost instantaneously by the cold-box process, using vaporous sulfur dioxide as the curing agent (most typically a blend of nitrogen, as a carrier, and sulfur dioxide containing from 35 weight percent to 65 weight percent sulfur dioxide),

described in U.S. Pat. Nos. 4,526,219 and 4,518,723, which are hereby incorporated by reference. The shaped article is preferably exposed to effective catalytic amounts of gaseous sulfur dioxide, and, optionally, a carrier gas can be used. The exposure time of the sand mix to the gas is typically from 0.5 to 10 seconds. The foundry shape is cured after gassing with sulfur dioxide. Oven drying may be needed if the foundry shape is coated with a refractory coating.

The core and/or mold may be formed into an assembly. When making castings, the assembly may be coated with a water-based refractory coating and passed through a conventional or microwave oven to remove the water from the coating.

## ABBREVIATIONS

The abbreviations used in the examples are as follows:

|             |                                                                                                                                                    |
|-------------|----------------------------------------------------------------------------------------------------------------------------------------------------|
| SCA         | silane coupling agent.                                                                                                                             |
| BT          | butyl ester of tall oil fatty acid, PLASTHALL 503 from CP Hall.                                                                                    |
| CHP         | cumene hydroperoxide.                                                                                                                              |
| 25 ERL-4221 | an aliphatic epoxy resin, 3,4-epoxycyclohexylmethyl 3,4-epoxy-cyclohexane-carboxylate, manufactured by Union Carbide.                              |
| HF          | as a 49 weight percent aqueous solution.                                                                                                           |
| TONE 0301   | caprolactone based trifunctional polyol with average molecular weight of 300 and a hydroxyl number of 560 mg KOH/g, manufactured by Union Carbide. |

## EXAMPLES

While the invention has been described with reference to a preferred embodiment, those skilled in the art will understand that various changes may be made and equivalents may be substituted for elements thereof without departing from the scope of the invention. In addition, many modifications may be made to adapt a particular situation or material to the teachings of the invention without departing from the essential scope thereof. Therefore, it is intended that the invention not be limited to the particular embodiment disclosed as the best mode contemplated for carrying out this invention, but that the invention will include all embodiments falling within the scope of the appended claims. In this application, all units are in the metric system and all amounts and percentages are by weight, unless otherwise expressly indicated.

### Testing Protocol

The various formulations given in the following examples were evaluated by preparing test cores whose tensile strengths were measured over various times. How well a binder system bonds the particles of an aggregate (e.g. sand) together is typically evaluated by using tensile strength measurements given in pounds per square inch (psi). Sufficient core strength is needed once the binder/sand mix is 60 cured to prevent the core/mold from distorting or cracking during assembly operations. Tensile strength measurements are taken immediately (20 seconds after core box opens), 5-minutes, one-hour, 24-hours and 24 hours at 90% relative humidity according to the standard ASTM sand tensile test. Cores made with binder systems that retain higher tensile strengths over time can better retain their dimensional accuracy and have less core breakage problems.

## Comparison Example A

A binder, having no acrylic component or HF, was used in this comparison example. The composition of the binder follows:

|               |        |
|---------------|--------|
| ERL 4221      | 57.57% |
| Butyl Tallate | 27.21  |
| CHP           | 15.02  |
| SCA           | 0.20   |

A foundry mix was prepared by mixing 3000 grams of silica sand and 30 grams of the 11 binder for 4 minutes using a Hobart sand mixer. The foundry mix was then blown into a three cavity tensile test specimen core box and gassed 0.5 second with a 65/35 SO<sub>2</sub>/nitrogen mixture delivered by an MT Systems SO<sub>2</sub>/Nitrogen blending unit followed by a 10 second dry air purge. The tensile strengths were measured according to standard ASTM measurements and are summarized in Table I.

## Example 1

Comparison Example A was repeated using the following binder, which contained HF:

|               |       |
|---------------|-------|
| ERL 4221      | 57.5% |
| Butyl Tallate | 27.18 |
| CHP           | 15.0  |
| SCA           | 0.20  |
| HF            | 0.12  |

The tensile strengths were measured according to standard ASTM measurements and are summarized in Table I.

## Example 2

Example 1 was repeated using the following binder, which contained a polyol in addition to HF:

|               |        |
|---------------|--------|
| ERL 4221      | 57.50% |
| TONE 0301     | 2.80   |
| Butyl Tallate | 24.38  |
| CHP           | 16.50  |
| SCA           | 0.20   |
| HF            | 0.12   |

The tensile strengths were measured according to standard ASTM measurements and are summarized in Table I.

TABLE I

| Example | Tensile strengths of cores (psi) |                 |                 |       |      |        | 24 hr @<br>95%<br>RH |
|---------|----------------------------------|-----------------|-----------------|-------|------|--------|----------------------|
|         | HF<br>(pbw)                      | Polyol<br>(pbw) | Imm<br>(20 sec) | 5-min | 1-hr | 24 hrs |                      |
| A       | 0                                | 0               | 87              | 134   | 166  | 164    | 81                   |
| 1       | 0.12                             | 0               | 98              | 162   | 189  | 188    | 116                  |
| 2       | 0.12                             | 2.80            | 74              | 123   | 133  | 154    | 146                  |

A comparison of Example A and Example 1 indicates that the addition of HF gives better sand tensile strengths, especially the 24-hour humidity resistance. Example 2 indicates that the addition of HF and a polyol (TONE 0301) to the acrylicate-free binder lowered the initial sand tensile strengths, but dramatically improved the humidity resistance by 80%, relative to the Comparison Example A.

Thus, the subject invention results in improvements that provide more flexibility to the foundryman. Besides simplifying the customer's binder-storage and handling operations, improvements in tensile strength development allow use of lower binder levels. This provides benefits in the casting of metal parts from both aluminum and ferrous metals.

15 We claim:

1. A foundry binder system, which will cure in the presence of sulfur dioxide and an oxidizing agent, comprising:

- (a) 45 to 80 parts by weight of an epoxy resin;
- (b) 5 to 40 parts of an ester of a fatty acid;
- (c) 0.05 to 3 parts of a fluorinated acid selected from the group consisting of hydrofluoric acid, ammonium bifluoride, tris-hydrofluoric acid, potassium bifluoride, N,N-diisopropyl-amine-tris (hydrogenfluoride), and N,N'-dimethyl-2-imidazolidone-hexakis(hydrogenfluoride);
- (d) from 10 to 40 parts by weight of an oxidizing agent; and
- (e) 0 parts of an ethylenically unsaturated monomer or polymer,

wherein (a), (b), (c), and (d) are separate components or mixed with another of said components, and where said parts by weight are based upon 100 parts of binder.

2. The binder system of claim 1 wherein the epoxy resin is selected from the group consisting of epoxy resins derived from bisphenol A, epoxy resins derived from bisphenol F, epoxidized novolac resins, cycloaliphatic epoxy resins, and mixtures thereof.

3. The binder system of claim 2 wherein the epoxy resin has an epoxide equivalent weight of about 165 to about 225 grams per equivalent.

4. The foundry binder system of claim 3 wherein the aqueous solution of fluorinated acid is an aqueous solution of hydrofluoric acid containing from 10 to 90 weight percent water.

5. The binder system of claim 4 wherein the oxidizing agent is cumene hydroperoxide.

6. The foundry binder system of claim 5 wherein the amount of epoxy resin is from 50 to 70 parts by weight, the amount of ester of a fatty acid is from 15 to 30, the amount of fluorinated acid is from 0.1 to 1.0, and the amount of oxidizing agent is from 12 to 30 parts by weight, where the weights are based upon 100 parts of the binder system.

7. The foundry binder system of claim 6 which further comprises a polyol.

8. A foundry mix comprising:

- (a) a major amount of foundry aggregate;
- (b) an effective bonding amount of the foundry binder system of claim 1, 2, 3, 4, 5, 6, or 7.

9. A cold-box process for preparing a foundry shape comprising:

- (a) introducing the foundry mix of claim 8 into a pattern; and
- (b) curing with gaseous sulfur dioxide.

10. A foundry shape prepared in accordance with claim 9.

- 11.** A process of casting a metal article comprising:  
(a) fabricating a foundry shape in accordance with claim  
**10;**  
(b) pouring said metal while in the liquid state into said  
foundry shape;

- (c) allowing said metal to cool and solidify; and  
(d) then separating the molded article.  
**12.** A casting prepared in accordance with claim **11.**

\* \* \* \* \*